

[54] MANUFACTURE OF SILVER-CADMIUM  
OXIDE WIRE

[75] Inventors: Loren Godfrey, Morristown;  
Krishnamurthy Vaithinathan,  
Edison, both of N.J.

[73] Assignee: Engelhard Minerals & Chemicals  
Corporation, Murray Hill, N.J.

[22] Filed: June 12, 1973

[21] Appl. No.: 369,317

[52] U.S. Cl..... 148/6.3, 148/11.5 R, 75/173 A,  
117/231

[51] Int. Cl..... C23c 11/00, C21d, C22c 5/00  
[58] Field of Search..... 148/6.3, 11.5 R; 75/173 A;  
117/231

[56] References Cited

UNITED STATES PATENTS

2,932,595 4/1960 Pflumm..... 148/11.5 R  
3,666,428 5/1972 Haarbye..... 75/173 A X

FOREIGN PATENTS OR APPLICATIONS

960,592 6/1964 Great Britain..... 75/173 A

Primary Examiner—John D. Welsh

[57] ABSTRACT

Pre-oxidized silver-cadmium oxide wire, such as pre-oxidized 90Ag 10CdO wire obtained by 91Ag 9Cd alloy wire, is prepared by plural stage oxidation. The silver-cadmium alloy wire is initially prepared having a diameter greater than the diameter of the finished wire  $D_f$ , e.g., in the range 1.7–2.0  $D_f$ . Following each oxidation operation comprising the plural stage oxidation the resulting oxidized wire is drawn or otherwise reduced in diameter, the desired finished diameter  $D_f$  being reached after the last oxidation operation. The oxidation operations making up the plural stage oxidation are carried out such that the matrix area of the finished wire is substantially 100% oxidized, i.e., the cadmium content of the wire is substantially completely oxidized to cadmium oxide.

22 Claims, 1 Drawing Figure

PATENTED FEB 25 1975

3,868,275

FLOW SHEET FOR MANUFACTURE OF 90 Ag 10 CdO  
PREOXIDIZED WIRE BY 3 STAGE OXIDATION PROCESS

$D_f$  = DIAMETER OF FINISHED WIRE  
91 Ag 9 Cd ALLOY

EXTRUDE OR CONTINUALLY CAST  
DRAW TO 1.7 - 2.0 TIMES  $D_f$

1ST STAGE OXIDATION - 1500-  
1540° F AIR OR OXYGEN ENRICHED  
AIR - 15-30% OF MATRIX AREA OXIDIZED  
1 - 8 HOURS

DRAW TO 1.5 - 1.8 TIMES  $D_f$

2nd STAGE OXIDATION - 1500° F AIR  
OR OXYGEN ENRICHED AIR 30-50%  
OF MATRIX AREA OXIDIZED  
4-16 HOURS

DRAW TO 1.2 - 1.5 TIMES  $D_f$

3rd STAGE OXIDATION - 1500° F  
IN AIR OR OXYGEN ENRICHED AIR  
100% MATRIX AREA OXIDIZED -  
ALLOY OF 91 Ag 9 Cd IS CONVERTED  
TO 90 Ag 10 CdO 24-64 HOURS

DRAW TO ABOUT  $(0.002" + D_f)$

ANNEAL - 1000° F - 1 HOUR

PICKLE DIL.  $H_2SO_4$

DRAW TO  $D_f$

## MANUFACTURE OF SILVER-CADMIUM OXIDE WIRE

This invention relates to the manufacture of pre-oxidized silver-cadmium oxide wire. More particularly, this invention is directed to the manufacture of pre-oxidized silver-cadmium oxide wire derived from internally oxidizable silver-cadmium alloys containing up to about 20% by weight cadmium.

Silver-cadmium oxide compositions have long been known to be useful for the manufacture of electrical contact elements and the like, see U.S. Pat. Nos. 2,307,668, 2,539,298, 2,796,346, 2,830,898, 2,932,595, 3,472,654, 3,477,845 and 3,666,428. The disclosures of each of the above-identified patents are herein incorporated and made part of this disclosure.

As indicated by the disclosures of the above-identified patents, there has been considerable interest in developing a satisfactory process for the preparation of pre-oxidized silver-cadmium oxide wire from silver-cadmium alloys. For the most part, however, the methods and techniques known heretofore for the production of a pre-oxidized silver-cadmium oxide wire have not been completely satisfactory. For example, techniques have been developed to produce a pre-oxidized silver-cadmium oxide wire but when such wire was headed to rivets for the production of electrical contact elements the resulting rivets were unsatisfactory due to cracking. In the methods known heretofore to produce pre-oxidized silver-cadmium oxide wire and the like, the oxidation process for the production of the pre-oxidized wire has usually been carried out in a single stage oxidation operation. As indicated hereinabove, however, completely satisfactory results were not obtained.

It is an object of this invention to provide an improved process for the manufacture of pre-oxidized silver-cadmium oxide wire useful for the manufacture of electrical contact elements therefrom, such as rivets and the like.

It is another object of this invention to provide an improved process for the oxidation of silver-cadmium alloys, such as silver-cadmium alloys containing up to about 20% by weight cadmium, for the manufacture of pre-oxidized silver-cadmium oxide materials, structures, strips or wire therefrom.

It is yet another object of this invention to provide an improved process for the preparation of pre-oxidized silver-cadmium oxide wire especially satisfactory for the production of rivets therefrom.

How these and other objects of this invention are achieved will become apparent in the light of the accompanying disclosure and particularly with reference to the accompanying drawing wherein there is illustrated a flow sheet for the manufacture of 90Ag 10Cd0 pre-oxidized wire in accordance with one preferred embodiment of the practices of this invention. In at least one embodiment of the practices of this invention at least one of the foregoing objects will be achieved.

In accordance with the practices of this invention there is provided a process for the manufacture of pre-oxidized silver-cadmium oxide compositions and structures, such as wire, derivable from internally oxidizable silver-cadmium alloys containing up to about 20% by weight cadmium. The practices of this invention are particularly applicable to the most common and typical internally oxidizable silver-cadmium alloy containing about 91% by weight silver and about 9% by weight

cadmium which is oxidizable to the composition 90% by weight silver and 10% by weight cadmium oxide.

Although emphasis is placed in the disclosure of this invention on silver-cadmium alloys containing up to 20% by weight cadmium, such as silver-cadmium alloys containing 5-15% by weight cadmium, the silver-cadmium alloy which is treated in accordance with this invention to provide silver-cadmium oxide compositions particularly useful for the manufacture of electrical contact elements might also include other metal additives up to about 10% by weight of the silver-cadmium alloy. Suitable such additives include cobalt, nickel, thallium, copper, potassium and calcium.

The internally oxidizable silver-cadmium alloy compositions in accordance with this invention are subjected to a plural stage oxidation operation in contact with air or oxygen-enriched air or oxygen at an elevated temperature and, if desired, at an elevated pressure, such as in the range 1-10 atm. abs. The oxidation operation is carried out in a plurality of separate oxidation operations sufficient to effect substantially 100% oxidation of the matrix, e.g., the wire matrix or cross-section of the silver-cadmium alloy, so as to convert substantially all of the cadmium content to cadmium oxide. The plural stage oxidation operation in accordance with this invention may comprise two separate oxidation operations or as many as six or more separate oxidation operations, depending upon the shape and/or thickness of the silver-cadmium alloy material or structure undergoing oxidation. Usually, a plural stage oxidation operation made up of three separate oxidation operations is sufficient to substantially completely convert the cadmium content of the silver-cadmium alloy material or structure undergoing oxidation to cadmium oxide.

The oxidation operations making up the plural stage oxidation treatment in accordance with this invention are usually carried out at an elevated temperature, preferably at a temperature of about 1,500°F., such as a temperature in the range 1,450°-1,550°F., more or less, about 1,200°F. or higher but below the melting point of the alloy undergoing oxidation, preferably at least about 25°F. below the melting point. The separate oxidation operations making up the plural stage oxidation treatment need not be carried out at the same temperature or with the same temperature range, although effective and satisfactory results have been achieved by carrying out the oxidation operations at a temperature in the range from about 1,450° to about 1,550°F. The individual oxidation operations making up the plural stage oxidation treatment are carried out for a period of time in the range from about 1 hour to about 100 hours, depending upon the cadmium content in the alloy undergoing oxidation. Also, depending upon the size and/or shape and/or thickness of the oxidation temperature and oxygen concentration and pressure employed, each separate oxidation operation might be satisfactorily completed within a rather short period of time, as low as 15-30 minutes, or might require a substantial period of time, such as high as 100 hours.

As indicated hereinabove, the internally oxidizable silver-cadmium alloy materials are subjected to a plural stage oxidation treatment which might be made up of two or more, such as six, separate oxidation operations. Each separate oxidation operation is carried out to effect a conversion of the cadmium of the silver-cadmium alloy material undergoing oxidation to cad-

mium oxide so that upon completion of the plural stage oxidation treatment substantially the entire cadmium content of the silver-cadmium alloy material undergoing treatment has been converted to cadmium oxide.

By way of example, and with reference to the preferred embodiment of the practices of this invention involving a three stage oxidation operation of silver-cadmium alloy wire, the first stage oxidation operation is carried out such that the matrix area of the silver-cadmium alloy wire is oxidized to about 15-30%, i.e., 15-30% of the cross-sectional area is oxidized such that the cadmium content therein is converted to cadmium oxide. In the second stage oxidation operation the matrix area would be oxidized to an even greater extent, to about 30-50% of the matrix area. In the third stage operation the matrix area would be 100% oxidized, i.e., the cadmium content of the silver-cadmium alloy wire would be substantially completely converted to cadmium oxide.

Depending upon the shape and/or composition of the silver-cadmium alloy material undergoing treatment, as indicated hereinabove, the plural stage oxidation operation may be carried out in as many as two separate oxidation operations or might require as many as six separate oxidation operations. Accordingly, in a two stage oxidation treatment the first stage oxidation operation might result in the oxidation of 40-80% of the matrix area, more or less, or as low as 5-15% of the matrix area in a six stage oxidation treatment. Upon completion of the plural stage oxidation operation, however, substantially 100% of the matrix area of the silver-cadmium alloy material undergoing treatment would be completely oxidized and converted to the corresponding silver-cadmium oxide composition.

Another feature in the practices of this invention, and particularly in the preferred embodiment thereof wherein silver-cadmium alloy wire is oxidized, after each separate oxidation treatment in the plural stage oxidation the silver-cadmium alloy material or structure or wire is reduced in cross-section so that the following oxidation treatment in the plural stage oxidation is operative upon the previously oxidized silver-cadmium alloy material now having a reduced cross-section. In the practices of this invention therefore the silver-cadmium alloy material undergoing treatment is supplied to the first stage oxidation operation with a cross-section substantially greater than the cross-section of the desired finished completely oxidized silver-cadmium oxide product. For example, the cross-sectional area of the silver-cadmium alloy material or structure initially subjected to the plural stage oxidation operation would have a cross-sectional area or average cross-sectional area substantially larger than the cross-sectional area in the finished product. Specifically, the cross-sectional area of the silver-cadmium alloy material supplied to the first stage oxidation operation of the plural stage oxidation might be as large as or greater than twice the cross-sectional area in the finished product, such as having a cross-sectional area in the range from 2 to 9 times larger in the cross-sectional area of the finished oxidized product.

Upon completion of the first stage oxidation operation the resulting oxidized silver-cadmium alloy material or structure or wire would be reduced in cross-section say from a value of 2 times the desired finished diameter in the case of wire to about 1.2-1.8 times the diameter of the finished wire. When this material has

been subjected to a second oxidation operation the resulting oxidized silver-cadmium material would be again reduced in cross-section, e.g., diameter in the case of wire, to about 1.1-1.5 times the diameter of the finished completely oxidized product wire. Upon the completion of a third stage oxidation treatment this twice reduced silver-cadmium alloy material would be again reduced in cross-sectional area to substantially that of the cross-section or diameter desired in the finished product. The thus-treated material after suitable annealing, if necessary, and pickling, if necessary, could then be finished or reduced in cross-section to the cross-section desired in the finished product.

As indicated hereinabove, each oxidation treatment is followed by a size reducing or drawing operation wherein the cross-sectional area of the previously oxidized silver-cadmium alloy structure is reduced. Upon the completion of the plural stage oxidation operation and the size reducing or drawing operation following the last oxidation operation the resulting oxidized silver-cadmium oxide structure would have a cross-sectional area corresponding substantially to that desired in the finished product.

Each reducing or drawing operation need not effect a reduction in cross-sectional area of the silver-cadmium alloy material undergoing treatment to the same extent. Greater or lesser reduction in cross-sectional area may be effected after the first or the last oxidation operation. In the overall practice of the invention, however, upon the completion of the plural stage oxidation treatment with the intermediate size reducing or drawing operations the resulting silver-cadmium product will substantially correspond in size to the size desired in the finished product and the cadmium content of the silver-cadmium alloy material initially supplied to the operation will be substantially converted or oxidized to cadmium oxide.

Reference is now made to the drawing which schematically illustrates by way of a flow sheet the preferred practice of this invention directed to the treatment of a silver-cadmium alloy wire having the composition 91% by weight silver and 9% by weight cadmium, the wire having a diameter in the range 1.7-2.0 times that of the diameter of the finished wire  $D_f$ . The 91Ag 9Cd alloy is either extruded or continuously cast and then drawn to about 1.7-2.0 times the required finished diameter. The first stage oxidation is carried out at 1,500°-1,540°F. in air or in oxygen-enriched air for a period of time such that about 15-30% of the matrix area is oxidized. The resulting partially oxidized wire is then reduced in diameter or drawn to 1.5-1.8 times the required finish size. The second stage oxidation operation is then carried out at a temperature of about 1,500°F. in air or in oxygen-enriched air for a period of time sufficient to effect oxidation of about 30-50% of the matrix area. The partially oxidized wire from the second stage oxidation is reduced in size or drawn to about 1.1-1.5 times the required finish diameter. Thereupon, the third stage oxidation operation is carried out at a temperature of about 1,500°F. in air or oxygen-enriched air to effect substantially complete or 100% oxidation of the matrix. Upon the completion of the third stage oxidation operation the original alloy of the composition 91Ag 9Cd is converted to the corresponding composition 90Ag 10Cd0. The resulting completely oxidized material is then cold worked, if necessary, annealed, such as by heating to a tempera-

ture of about 1,000°F. and then drawn to the required finish temper. The resulting wire is then pickled in dilute sulfuric acid, if necessary.

Wire prepared in accordance with the practices of this invention and having the composition 90Ag 10Cd0 was tested for headability, i.e., rivet formation therefrom. The wire produced in accordance with this invention had good headability and had a very small crack rate, if any, in the head to shank diameter ratios normally prepared. The degree of grain boundary Cd0 precipitation was also found to be minimum, if any. It would appear that the better mechanical properties, good ductility and headability in rivet manufacture of this wire might be due to the "sound" matrix of the alloy. It also appears that the intermediate cold working and oxidation refines the grain size. The presence of cadmium oxide in the matrix seemed to slow down the grain growth of the matrix and helps in strengthening the matrix. Short cycle of oxidation time seems to eliminate cracking of the oxidized wire and the width of interruption bands of oxidation seen in the thus-produced wire where cadmium oxide composition may be deviated from "average composition" is very small. In a typical case there was found to be about 0.0004 inch. This could be minimized by altering oxygen potential, temperature or cooling rate in a subsequent oxidation.

Wire produced in accordance with the practices of this invention as illustrated in the preferred embodiment shown in the drawing provides a superior wire, especially for rivet manufacture.

Further illustrative of the practices of this invention there are set forth in accompanying Table No. 1 procedures for the preparation of preoxidized silver-cadmium oxide wire in accordance with the practices of this invention:

Table No. 1

## OXIDATION PROCEDURES FOR Ag-9%-Cd WIRE

|                   | A                    | B                    | C                    | D                    |
|-------------------|----------------------|----------------------|----------------------|----------------------|
| Starting Diameter | .095"                | .135"                | .155"                | .195"                |
| Oxidize           | 1540°F.,<br>1½ hour  | 1540°F.,<br>2½ hours | 1540°F.,<br>5 hours  | 1540°F.,<br>8 hours  |
| Draw to           | .080"                | .115"                | .135"                | .165"                |
| Oxidize           | 1500°F.,<br>4 hours  | 1500°F.,<br>6 hours  | 1500°F.,<br>11 hours | 1500°F.,<br>16 hours |
| Draw to           | .070"                | .100"                | .115"                | .130"                |
| Oxidize           | 1500°F.,<br>24 hours | 1500°F.,<br>40 hours | 1500°F.,<br>48 hours | 1500°F.,<br>64 hours |
| Use for Sizes     | .062"                | .090-.063"           | .105-.090"           | .120-.105"           |
|                   | and below            |                      |                      |                      |

Typical properties of the resulting preoxidized silver-cadmium oxide wire are set forth in accompanying Table No. 2:

Table No. 2

## TYPICAL PROPERTIES OF PREOXIDIZED Ag-10% CdO WIRE

| Condition            | T.S. (Ksi) | Elong. (2" gauge) |
|----------------------|------------|-------------------|
| As oxidized          | 25-35      | 40-60%            |
| Annealed 1000°F.     | 25-35      | 40-60%            |
| .002" Hard           | 30-40      | 25-45%            |
| Typical Analysis:    |            |                   |
| CdO: 10% $\pm$ 1.0   |            |                   |
| Impurities: .15 Max. |            |                   |
| Ag: Balance          |            |                   |

As will be apparent to those skilled in the art in the light of the foregoing disclosure, many alterations, modifications and substitutions are possible in the practice of this invention without departing from the spirit or scope thereof.

We claim:

1. A method for the manufacture of silver-cadmium oxide wire having the diameter  $D_f$  which comprises forming from silver-cadmium alloy wire having the diameter from about 1.5 to about  $3 D_f$ , subjecting the resulting formed wire to a first stage oxidation at a temperature in the range from about 1,450° to about 1,550°F. in contact with air or oxygen-enriched air or oxygen for a period of time to effect oxidation of the wire to about 15-30% of the matrix area thereof, drawing the resulting first stage oxidized wire to a diameter in the range from about 1.2 to about  $2 D_f$ , subjecting the thus-drawn first stage oxidized wire to a second stage oxidation at a temperature in the range 1,450°-1,550°F. in contact with air or oxygen-enriched air or oxygen for a period of time sufficient to effect oxidation of about 30-50% of the matrix area thereof, drawing the wire resulting from the second stage oxidation to a diameter in the range 1.1-1.5  $D_f$ , subjecting the thus-drawn second stage oxidized wire to a third stage oxidation at a temperature in the range 1,450°-1,550°F. in contact with air or oxygen-enriched air or oxygen until 100% of the matrix area of the wire has been oxidized, subjecting the resulting third stage oxidized wire to drawing to about  $D_f$ .
2. A method in accordance with claim 1 wherein the silver-cadmium alloy wire contains about 5-15% cadmium by weight.
3. A method in accordance with claim 1 wherein the silver-cadmium alloy has the composition of about 91% by weight silver and about 9% by weight cadmium and

wherein the oxidized wire resulting from the third stage oxidation has a composition of about 90% by weight silver and about 10% by weight cadmium oxide.

4. A method in accordance with claim 1 wherein the first stage oxidation is carried out for a period of time in the range from about 1 to about 8 hours.
5. A method in accordance with claim 1 wherein said first stage, said second stage and said third stage oxidation operations are carried out for a period of time in the range from about 1-8 hours, 4-16 hours and 24-64 hours, respectively.
6. A method in accordance with claim 1 wherein the wire resulting from the third stage oxidation operation and after drawing to about  $D_f$  is subjected to annealing at a temperature of about 1,000°F.

7. A method in accordance with claim 1 wherein said first stage, said second stage and said third stage oxidation operations are carried out in contact with air.

8. A method for the manufacture of silver-cadmium oxide wire having the diameter  $D_f$ , which comprises forming silver-cadmium alloy wire having a diameter greater than  $D_f$ , subjecting the resulting formed wire to plural stage oxidation in contact with air or oxygen-enriched air or oxygen with intermediate drawing of the resulting oxidized wire wherein after each oxidation stage the wire is reduced in diameter until the desired diameter  $D_f$  is reached, each stage of said plural stage oxidation being carried out at a temperature in the range from about 1,200°F. to a temperature at least about 25°F. below the melting point of said silver-cadmium alloy and for a period of time in the range from about 15 minutes to about 100 hours, the plural stage oxidation being carried out so as to effect substantially complete oxidation of the cadmium present in the cadmium alloy wire to cadmium oxide.

9. A method in accordance with claim 8 wherein the silver-cadmium alloy wire has a diameter in the range 1.5-3  $D_f$ .

10. A method in accordance with claim 8 wherein said silver-cadmium alloy contains up to 20% by weight cadmium.

11. A method in accordance with claim 8 wherein said plural stage oxidation comprises two separate oxidation operations.

12. A method in accordance with claim 8 wherein said plural stage oxidation comprises three separate oxidation operations.

13. A method in accordance with claim 8 wherein said plural stage oxidation comprises four separate oxidation operations.

14. A method in accordance with claim 8 wherein said plural stage oxidation comprises five separate oxidation operations.

15. A method in accordance with claim 8 wherein the initial stage oxidation of said plural stage oxidation includes an oxidation operation wherein the silver-cadmium alloy wire is subjected to contact with air or oxygen-enriched air or oxygen at a temperature in the range from about 1,450° to about 1,550°F. for a period of time in the range from about 1 to 8 hours.

16. A method in accordance with claim 8 wherein immediately following the last oxidation stage making

up the plural stage oxidation the wire is drawn to the desired diameter  $D_f$ .

17. A method in accordance with claim 8 wherein immediately following the last oxidation stage making up the plural stage oxidation the resulting oxidized wire is drawn to a diameter slightly larger than the desired diameter  $D_f$ , followed by annealing and pickling the resulting drawn oxidized wire and then drawing the wire to the desired diameter  $D_f$ .

18. A method for the manufacture of a silver-cadmium oxide structure having an average cross-sectional area A from a silver-cadmium alloy containing up to about 20% by weight cadmium which comprises forming a silver-cadmium alloy structure having an average cross-sectional area B from said silver-cadmium alloy, B being greater than A, subjecting the resulting formed silver-cadmium alloy structure to plural stage oxidation in contact with air or oxygen-enriched air or oxygen to effect upon completion of the last oxidation stage substantially 100% oxidation of the cadmium content of said cadmium alloy structure to cadmium oxide, each stage of said plural stage oxidation being carried out at a temperature in the range from about 1,200° to about 25°F. below the melting point of said silver-cadmium alloy and for a period of time in the range from about 15 minutes to about 100 hours, during said plural stage oxidation there being at least one intermediate size reduction of the oxidized silver-cadmium alloy structure wherein the structure is substantially reduced in cross-sectional area to a value intermediate B and A and upon completion of the plural stage oxidation reducing the cross-sectional area of the silver-cadmium oxide structure to the desired cross-sectional area A.

19. A method in accordance with claim 18 wherein the plural stage oxidation operation comprises a plurality of separate oxidation operations from two to six in number.

20. A method in accordance with claim 18 wherein said silver-cadmium alloy contains up to about 10% by weight of an additive metal or oxide thereof based on said silver-cadmium alloy.

21. A method in accordance with claim 18 wherein said silver-cadmium alloy structure is a strip or bar.

22. A method in accordance with claim 18 wherein said silver-cadmium alloy structure is wire.

\* \* \* \* \*